



US007895874B2

(12) **United States Patent**  
Mathai et al.

(10) **Patent No.:** US 7,895,874 B2  
(45) **Date of Patent:** Mar. 1, 2011

(54) **NEAR NET SHAPE FORGING PROCESS FOR COMPRESSOR AND TURBINE WHEELS AND TURBINE SPACER WHEELS**

(75) Inventors: **Manu Mathai**, Chennai (IN); **Raymond Stonitsch**, Simpsonville, SC (US); **Guven Yucesan**, Greenville, SC (US)

(73) Assignee: **General Electric Company**, Schenectady, NY (US)

(\*) Notice: Subject to any disclaimer, the term of this patent is extended or adjusted under 35 U.S.C. 154(b) by 478 days.

(21) Appl. No.: **11/968,684**

(22) Filed: **Jan. 3, 2008**

(65) **Prior Publication Data**

US 2009/0173132 A1 Jul. 9, 2009

(51) **Int. Cl.**

**B21D 22/00** (2006.01)

**B21K 25/00** (2006.01)

**B23P 15/04** (2006.01)

(52) **U.S. Cl.** ..... **72/357; 72/353.2; 72/403; 29/889.2**

(58) **Field of Classification Search** ..... 72/352, 72/356, 357, 377, 105, 118, 120, 121, 260, 72/353.2, 353.6, 360, 399, 402, 403; 29/889.2, 29/889.23, 889.7; 100/35, 42

See application file for complete search history.

(56) **References Cited**

**U.S. PATENT DOCUMENTS**

5,950,481 A 9/1999 Sarkisian et al.  
6,240,765 B1 6/2001 Delgado et al.

*Primary Examiner*—Teresa M Bonk

(74) *Attorney, Agent, or Firm*—Nixon & Vanderhye P.C.

(57) **ABSTRACT**

A method of forging a workpiece includes (a) incrementally advancing the workpiece in a closed die forge, the closed die forge including a stationary, flat die and a first split die including a plurality of first die segments, each die segment being incrementally advanced in sequence to contact the incrementally advancing workpiece; (b) replacing the stationary, flat die with a second split die including a plurality of second die segments; and (c) forging the workpiece forged in (a) between the first split die and the second split die, wherein the first die segments are stationary and at least some of the plurality of second die segments are incrementally advanced in sequence.

**10 Claims, 6 Drawing Sheets**





FIG. 2



FIG. 3



FIG. 1



FIG. 5



FIG. 6



FIG. 4





FIG. 10



FIG. 9



FIG. 12



FIG. 11



**FIG. 13**

## NEAR NET SHAPE FORGING PROCESS FOR COMPRESSOR AND TURBINE WHEELS AND TURBINE SPACER WHEELS

The invention relates to a near net shape forging process for compressor and turbine wheels and turbine spacer wheels. In particular, the invention relates to a near net shape forging process for compressor and turbine wheels and turbine spacer wheels formed of NiCrMoV and CrMoV.

### BACKGROUND OF THE INVENTION

Existing forging processes for the manufacture of compressor and turbine wheels rely on open die forging. Open die forging processes require additional input material tonnage and more heat treatment, and more forging processing steps.

Current closed die forging processes involve higher press tonnages. The use of closed die forging requires investments of higher capacity presses. However, there are currently no high capacity presses suitable for economical closed die forging of turbine and compressor wheels and turbine spacer wheels formed, for example, of CrMoV and NiCrMoV.

U.S. Pat. No. 6,240,765 discloses a closed die forging process including a die set having a stationary die and a movable die in facing-but-spaced-apart relation to the stationary die along a press access and defining a work piece volume therebetween. U.S. Pat. No. 6,240,765 starts with a workpiece geometry which covers the entire plan view area of the dies. As the workpiece covers the entire plan view area of the dies, the strain rates to be used are much lower which results in frequent heat treatment steps between the various incremental forging steps. The process of U.S. Pat. No. 6,240,765 therefore requires greater input material tonnage.

### BRIEF DESCRIPTION OF THE INVENTION

According to an embodiment of the invention, a method of forging a workpiece comprises (a) incrementally advancing the workpiece in a closed die forge, the closed die forge comprising a stationary, flat die and a first split die comprising a plurality of first die segments, each die segment being incrementally advanced in sequence to contact the incrementally advancing workpiece; (b) replacing the stationary, flat die with a second split die comprising a plurality of second die segments; and (c) forging the workpiece forged in (a) between the first split die and the second split die, wherein the first die segments are stationary and at least some of the plurality of second die segments are incrementally advanced in sequence.

According to another embodiment of the invention, a forging method comprises extruding a billet to form a ring shaped hollow workpiece; reducing a cross section of the workpiece; and forging the workpiece in a closed die comprising a first split die comprising a plurality of first die segments and a second split die comprising a plurality of second die segments.

### BRIEF DESCRIPTION OF THE DRAWINGS

FIG. 1 schematically illustrates the input material for a compressor or turbine wheel according to the prior art and the invention;

FIG. 2 depicts a first stage preforming process using a flat bottom die and a split top incremental die;

FIG. 3 discloses an incremental advance of a die segment from FIG. 2;

FIG. 4 discloses another advance of an incremental die segment of the first stage preforming;

FIGS. 5 and 6 show third stage preforming using the flat bottom die and incremental split top die;

FIGS. 7 and 8 schematically depict the fourth stage preforming with the flat bottom die and incremental split top die;

FIGS. 9 and 10 schematically depict the fifth stage preforming with a split bottom die and a stationary top die;

FIG. 11 schematically depicts sixth stage preforming with a split bottom die and a stationary top die;

FIG. 12 schematically depicts a turbine spacer wheel; and

FIG. 13 schematically depicts a forging process according to another embodiment of the invention.

### DETAILED DESCRIPTION OF THE INVENTION

Referring to FIG. 1, a turbine or compressor wheel 2 may be forged from a starting workpiece. According to current forging processes, the starting workpiece 4 comprises approximately 30% more material than a starting workpiece 6 according to an embodiment of the invention.

Referring to FIGS. 2 and 3, the first stage preforming may be performed with a closed flat bottom die 14 and a closed top incremental split die 16. The closed top incremental split die 16 includes a closed top die first segment 18, second segment 20, third segment 22, fourth segment 24, and a fifth segment 26. It should be appreciated, however, that the closed top incremental split die may be formed of any number of segments. A stop 40 is provided after the closed top die fifth segment 26 to close the die.

As shown in FIG. 2, the workpiece 6 is initially contacted by the first segment 18 and the second segment 20. The first segment 18 is incrementally advanced as shown in FIG. 3. The first stage preforming shown in FIGS. 4 and 5 is done at a high strain rate such as to minimize die chilling to avoid intermediate reheat of the workpiece 6.

The closed top die second segment 20 is then incrementally advanced, as shown in FIG. 4. The process details may be designed to eliminate the requirement for an intermediate reheat of the workpiece 6.

Referring to FIGS. 5 and 6, in a third stage of the preforming using the flat bottom die 14 and the top incremental split die 16, the third segment 22 is advanced to contact the workpiece 6. The third stage preforming process shown in FIGS. 5 and 6 is done at a high strain rate so as to minimize die chilling and avoid intermediate reheat processing of the workpiece 6.

As shown in FIGS. 7 and 8, the fourth stage preforming using the flat bottom die 14 and the top incremental split die 16 is shown. The fourth segment 24 is advanced to contact the workpiece 6 as shown in FIGS. 7 and 8.

As shown in FIGS. 2-8, the four preforming stages include incremental advancements of the first segment 18, the second segment 20, the third segment 22, and the fourth segment 24 of the closed top incremental split die 16 against the flat bottom die 14. The four preforming stages are carried out at high strain rates to eliminate the intermediate heat treatment of the workpiece 6.

As shown in FIGS. 9 and 10, in a fifth stage of the preforming of the workpiece 6, the stationary flat bottom die 14 is replaced by a closed bottom incremental split die 28. The closed bottom incremental split die 28 includes a closed bottom die first segment 30, a second segment 32, a third segment 34, a fourth segment 36, and a fifth segment 38. The stop 40 is provided after the closed top incremental split die fifth segment 26 and the closed bottom die fifth segment 38 to provide a closed die.

As shown in FIGS. 9 and 10, the segments 18, 20, 22, 24, 26 of the closed top split die 16 remain stationary and the segments 30, 32, 34, 36, 38 of the closed bottom incremental

split die **28** are advanced to further shape the workpiece **6**. As shown in FIG. 15, the second segment **32** of the bottom die **28** is incrementally advanced. A heat treatment may be done on the workpiece **6** after the fifth stage preforming to bring the workpiece **6** back to temperature.

In the sixth stage preforming, shown in FIG. 11, the fourth segment **36** of the closed bottom incremental split die **28** is advanced. The sixth stage preforming is done at a very slow strain rate to minimize the load requirements.

As shown in FIGS. 2-11, the incremental forging of the compressor and/or turbine wheels may be performed in six preforming stages. The process shown in FIGS. 2-11 may be implemented across all of the frames and stages of the compressor and/or turbine. As the rotors have a significant length in the plan view area, the multistage and multi-preforming forging schedule shown in FIGS. 2-11 may be employed. In the first four preforming stages, the material of the workpiece **6** first flows primarily in the plan view direction using the bottom flat stationary die **14** and the top incremental split die **16** at high strain rates. The incremental forging is then completed in the fifth and sixth preforming stages using the bottom incremental split die **28** and the top incremental split die **16** at slower strain rates.

The top and bottom incremental split dies may be designed so that they are modular. For example, the bore-web sections are similar for stages **2-16** of compressor wheels, rim-web sections are similar between stages **10-16** and stages **2-5**. Variable rim-web sections for stages **6-9** can be represented by minimum web geometry. This permits the same basic die set to be used for various stages of wheels with minimum modifications without having the need to invest in a new die set for each stage of compressor/turbine wheels. The split die design enables a modular die design across various stages of GT wheels.

As the dies are at a lower temperature compared to the workpiece, having a thin plate made of a low thermal conductivity material at the interface between the dies and the workpiece is beneficial. This is more beneficial at the last stages of forging which are done at lower strain rates. This is desirable because die-chilling effect at the last stage could be high (due to the lower strain rates) leading to higher heat loss in the workpiece. Thus, having a thin lower conductivity material plate helps to reduce die chilling and thereby reduce the load requirements substantially.

FIG. 12 schematically depicts a turbine spacer wheel **42** which may be forged to near net shape according to an embodiment of the invention.

A billet having an initial diameter may be extruded in a die and mandrel arrangement with a container. The billet is forced through a mandrel and a punch and is shaped by an outer die including a container.

The geometry of the starting workpiece for the turbine spacer wheel may be a ring-shaped hollow profile. Such a workpiece reduces the load requirements of the incremental forging process. To achieve the ring-shaped profile, the mandrel extrusion process described above may be used. The use of mandrel extrusion for forming the workpiece starting geometry also permits subsequent drilling of the solid workpiece at the end of forging.

At the end of the extrusion process, a portion of the billet between the mandrel and the outer die and punch may be machined off to form the starting workpiece. The starting workpiece may be then used for the subsequent forging steps previously described.

Referring to FIG. 13, the turbine spacer wheel **42** may be forged by the closed top incremental split die **16** and the closed bottom incremental split die **28**. A shrink ring **52** may

be shrink fitted onto the stop **40**. The first segments **18, 30** are incrementally advanced toward one another. The second segments **20, 32** are then incrementally advanced toward one another. After incremental advancement of the first segments **18, 30**, a reheat may be performed on the workpiece **6** to raise the temperature of the workpiece.

In the third and fourth preforming stages, the third die segments **22, 34** are incrementally advanced towards one another and the fourth die segments **24, 36** are incrementally advanced toward one another.

The forging of the turbine spacer wheel as described requires only one reheat cycle in the incremental forging process which may be performed after the incremental advancement of the first segments **18, 30**.

Die stress analysis may be carried out after the forging process to estimate the die life. The maximum forces and stresses from the forged spacer wheel may be mapped onto the individual dies. During the forging of the turbine spacer wheel, the stop **40**, which is used to control the flow of the workpiece **6**, was subjected to high bursting stresses. It was also observed that a region **56** in each of the second segments **20, 32** was subjected to a very high tensile stress. The region is near the a fillet at the top region of the second segments **20, 32**. The remainder of the second segments **20, 32**, for example 95%, were in a safe compressive stress zone.

The forging process for forming the turbine spacer wheel may also be performed using the shrink ring **52** in place of the stop **40**. In that case, the fillet region of the second segments **20, 32** were subject to less tensile stress than in the forging process using only the stop **40**. As the remainder, e.g., 95% of the die regions remain in a state of compressive stress, the life of the dies is improved.

The closed die forging processes described above have been developed to permit the load requirements to be within the existing press requirement of 6 kton. The closed die forging processes described herein thus may be used with existing presses, which may have a capacity of 7 kton.

As there are currently no available closed die forgers for CrMoV and NiCrMoV compressor and turbine wheels, the use of the closed die forging processes described herein will allow use of existing forgers and provide better material properties and fracture appearance transition temperature (FATT) values. It should be appreciated, however, that other alloys may be used.

The closed die forging processes described herein also eliminate much of the required subsequent machining after the forging and thus provide a material savings of approximately 30%.

The use of the stop for restricting the material flow at the exit end of the dies permits the compressor and/or turbine wheels to be manufactured with a very high shaped difficulty factor. In addition, the use of die stress analysis to design and optimize the stop provides for a suitable shrink ring which increases the life of the stop.

The use of the incremental split dies described herein also permits the use of a modular die design across all of the stages of the compressor and/or turbine wheels. This permits the same setup of dies to be extended across all of the stages without the need for providing a new die set for each stage. This permits the same basic modular die set to be used for all of the stages and frames of the compressor and turbine wheels.

Closed die forgings are carried out both in open air and under protective atmosphere. The closed die forging processes described herein permits the forging and heat treat-

ment processes to be performed in air due to the die and/or workpiece geometry. This permits the use of less expensive die materials.

The preform shapes at the intermediate stages are also chosen such that the flow of the material of the workpiece **6** is primarily in one direction. The advantages of an open die configuration are thus available within the closed die described herein. This allows a lowering of the press requirements for use of a closed die.

The strain rates may also be chosen such that cooling of the workpiece is minimal. The strain rates may also be chosen so as not to increase the press requirements.

The geometry of the starting workpiece for the compressor and turbine wheels does not cover the entire plan view area of the dies. This permits the advantages of open die geometry to be obtained using a closed die. The closed die forging processes described herein may thus be thought of as a form of hybrid forging.

The geometry of the starting workpiece of the turbine spacer wheel may be a ring-shaped hollow profile. The geometry of the starting workpiece may be obtained by extrusion with a mandrel and container as described herein. The use of the hollow billet for forming the starting workpiece has at least two advantages, including, but not limited to, reducing the input material tonnage and eliminating subsequent machining. The use of the hollow billet to form the starting workpiece also reduces the load requirement during the near net shape forging.

Although the embodiments have been described in the context of forging compressor and turbine wheels and turbine spacer wheels, it should be appreciated that the process described herein may be used to forge other components, for example steam turbine rotors.

While the invention has been described in connection with what is presently considered to be the most practical and preferred embodiment, it is to be understood that the invention is not to be limited to the disclosed embodiment, but on the contrary, is intended to cover various modifications and equivalent arrangements included within the spirit and scope of the appended claims.

What is claimed is:

1. A method of forging a workpiece, comprising the steps of:
  - (a) incrementally advancing the workpiece in a closed die forge, the closed die forge comprising a stationary, flat die and a first split die comprising a plurality of first die segments, each die segment being incrementally advanced in sequence to contact the incrementally advancing workpiece;
  - (b) replacing the stationary, flat die with a second split die comprising a plurality of second die segments; and
  - (c) forging the workpiece forged in step (a) between the first split die and the second split die, wherein the first die segments are stationary and at least some of the plurality of second die segments are incrementally advanced in sequence.
2. A method according to claim 1, further comprising heat treating the workpiece in between advancement of at least some of the plurality of second die segments.
3. A method according to claim 1, wherein strain rates of the workpiece during step (a) are higher than strain rates of the workpiece during step (c).
4. A method according to claim 1, wherein a velocity of the first die segments during step (a) are higher than a velocity of the second die segments during step (c).
5. A method according to claim 1, wherein the workpiece does not initially cover an entire plan view area of the stationary, flat die and the first split die.
6. A method according to claim 1, wherein the workpiece is formed of CrMoV or NiCrMoV.
7. A method according to claim 1, wherein the first and second die segments are modular.
8. A method according to claim 7, wherein the modular die segments are configured to forge the workpiece into compressor or turbine wheels.
9. A method according to claim 8, wherein the compressor or turbine wheels comprise compressor or turbine wheels from each stage of a compressor or turbine.
10. A method according to claim 1, further comprising providing a thin plate of low thermal conductivity at an interface of the die segments and the workpiece during step (c).

\* \* \* \* \*